

Sept. 2, 1952

F. R. QUINN

2,609,470

RESISTANCE MATERIALS AND ELEMENTS

Filed July 22, 1949

Fig. 1.



Fig. 2. 4



Fig. 3.



Fig. 4.



Fig. 5a.



Fig. 6.



Fig. 7.



Fig. 8.



Inventor:  
Frederic R. Quinn,  
by *Andrew Cohen*  
His Attorney.

## UNITED STATES PATENT OFFICE

2,609,470

## RESISTANCE MATERIALS AND ELEMENTS

Frederic R. Quinn, Schenectady, N. Y., assignor  
to General Electric Company, a corporation of  
New York

Application July 22, 1949, Serial No. 106,293

34 Claims. (Cl. 201—63)

## 1

The present invention relates to resistance materials and elements and more particularly to metal-sulfide resistance materials and elements.

The invention is predicated on the discovery that resistance elements and materials characterized by a high degree of chemical stability and stability of resistivity can be obtained by utilizing compositions containing as essential ingredients at least two different metal sulfides, including molybdenum sulfide and a sulfide of a metal of group II of the periodic table.

It has been known that various compounds of metals, more specifically the oxides, sulfides, and selenides, or mixtures thereof possess certain desirable electrical resistance characteristics which make them particularly attractive for various applications in which a semi-conducting material is required. As many of the compounds or mixtures have also been characterized by a resistance which varies with changes in temperature, they have been used in regulating and protective systems as, for example, for temperature control purposes. However, the sulfide compositions known heretofore have been relatively unsatisfactory due to their inherent instability, particularly when subjected to elevated temperatures.

One object of the present invention is to provide stable sulfide resistance materials and elements.

Another object of the invention is to provide metal sulfide resistance materials and elements which are characterized by a high degree of chemical stability and stability of resistivity when subjected to wide variations in temperature.

A further object of the present invention is to provide a process for stabilizing the electrical characteristics of metal sulfide resistance elements.

Other objects and features of the present invention include additions for enhancing or improving the properties of the elements, such as additions of free sulfur, selection of suitable leads, the preparation of the elements and the treatment of the elements by a process designed to stabilize their electrical characteristics particularly for use in direct-current circuits. These specific features are hereinafter described, and further illustrated by examples of the preparation of certain elements, which examples are intended to set forth more specifically how the various aspects of the present invention are carried into effect.

The above and additional objects and features will become apparent from the following description taken in connection with the accompanying drawing wherein Figs. 1-5a inclusive are

cross-sectional views and Fig. 5b an end view of various forms of elements embodying the present invention; and Figs. 6-8 inclusive illustrate the temperature-resistance characteristics obtainable in certain of the products of the present invention.

While the elements of the present invention may be provided in any of a number of forms, a simple form of element of the thermistor-type is shown in Fig. 1 in which numeral 1 indicates a body of a mixture of metal sulfides including at least one of the group II metal sulfides with the ends of the leads 2 and 3 embedded in opposite ends of the body 1.

15 A modification of the element of Fig. 1 is shown in Fig. 2 wherein the sulfide body 4 is enclosed within and sealed into a glass housing 5 with the leads 6 and 7 extending through the opposite ends of the housing. The envelope 5 provides both physical and chemical protection for the sulfide element 4.

20 In Fig. 3, the electrical contacts 8 and 9 are shown in the form of caps which may be pressed onto the sulfide body 10 during the pressing operation. These cap-shaped contacts encompassing portions of the sulfide elements are respectively connected to lead wires 11 and 12 which may be any electrical conductor, such as a copper or nickel wire, soldered or welded or otherwise suitably connected to the contacts 8 and 9.

25 In Fig. 4, there is shown a self-contained element in which one of the contacts 14 is in the form of a case with the sulfide composition 15 pressed in the case and sintered in situ. In this modification, the second lead 16 is in the form of a wire having a flattened end portion 17 to provide additional anchoring means for the lead and increased contact surface with the sulfide mixture 15. The upper or open end of the casing 14 can be sealed by means of any suitable sealing material 19. A heat hardenable silicone resin is particularly useful for this purpose both because of its temperature resistance and because of the fact that it forms a heat resistant glassy exterior surface. Electrical contact may be made directly with the case 14 or by means of a suitable lead 18 connected thereto.

30 An element of the design shown in Figs. 5a and 5b is especially suited for many applications where a quick temperature response, particularly to radiant energy, is required. In this element the sulfide body 20 is generally flat but is provided with enlarged end portions 21 about leads 22 to obtain the desired conductivity adjacent the contacts. Due to the high ratio of surface

area to total mass, this modification has a relatively quick response to any change in temperature of the surroundings.

### Sulfides

The present invention is primarily based on the discovery that pressed, and preferably sintered, mixtures of metal sulfides essentially including at least one sulfide of a metal of group II of the periodic table, particularly a sulfide of magnesium, calcium, cadmium, zinc, barium or mercury, are characterized by a time and temperature stability much greater than exhibited by any of the known metal sulfide compositions. More specifically, the products of the present invention comprise a resistance or semi-conducting body consisting essentially of at least one group II metal sulfide hereinafter referred to as the "essential" sulfide, and at least one additional metal sulfide referred to hereinafter as the "base" sulfide or sulfides. The base sulfide may or may not be a group II metal sulfide. In addition to the essential and base sulfides, the resistance bodies of the invention also preferably include small amounts of molybdenum sulfide or sulfur or both. Further aspects of the invention include the combination of the sulfide bodies with contacts or leads of a particular type and the processing of the combination to provide an element having stable electrical characteristics for both A.-C. and D.-C. applications.

#### Essential and base sulfides

Ordinarily the essential sulfide is present in an amount ranging from about 3 to 95 percent, generally at least about 10 percent, by weight of the sulfide mixture. The preferred content of the essential sulfide is dependent upon the particular sulfides employed in making the elements. The primary function of the essential sulfide is to provide a composition which is stable and will exhibit the same resistance characteristics, i. e., will have the same resistance at any given temperature, over long periods of time or when repeatedly subjected either to sub-zero temperatures or heated to elevated temperatures up to and including those temperatures at which the single sulfides or mixtures of sulfides not containing one of the essential sulfides change their resistance characteristics generally as a result of the release or liberation of sulfur. Not only are the electrical characteristics of the products of the present invention stable, but they are also reproducible from batch to batch. The sulfur of the sintered polysulfide mixtures or alloys does not appear to be liberated even when the temperature of the products is raised to or above the evaporation temperature of sulfur.

All of the compositions and electrical elements of the present invention have resistance characteristics which change markedly with change in temperature. Practically all of them have substantial negative coefficients of electrical resistance. By proper selection of the alloying sulfides and the proportions thereof, products may be prepared which either have a constant or substantially constant decrease in resistance with increased temperature or which exhibit a sharp break in electrical resistance at a certain critical temperature, or narrow range of temperatures, the break-point temperature depending upon the composition of the metallic sulfide mixture and to a lesser extent upon the particular process employed in making the resistance element. Examples of sulfide mixtures which in cer-

tain proportions exhibit such sharp breaks in their resistance-temperature curves are silver calcium sulfide with a break temperature of around 175° C., and copper calcium sulfide with a break temperature slightly below 90° C. Molybdenum calcium sulfide mixtures can be prepared having break temperatures anywhere from 250 to 400° C. depending upon proportions used.

For any given application, the choice of a particular essential sulfide or sulfides will depend upon a number of factors. When the product is to operate at temperatures less than 500° C., the generally less expensive calcium, cadmium or magnesium sulfides are preferred. Calcium sulfide has the further advantage in that mixtures including it have very low temperature coefficients of expansion. If higher temperatures are to be encountered, the sulfide of mercury, and particularly the sulfides of zinc or barium should be used since polysulfide compositions containing these essential sulfides are stable at temperatures up to 1200° C. Cadmium sulfide compositions in general exhibit comparatively sharp break points, and steep temperature-resistance curves with calcium sulfide ranking next to the cadmium sulfide in this respect. Calcium sulfide exhibits no break temperature of its own so that the temperature-resistance characteristics, and particularly the break-point temperature of compositions containing this sulfide, will be primarily those of the base sulfide. The remaining essential sulfides all have their individual break-point temperatures and many of the compositions including these sulfides may have temperature-resistance curves with a plurality of break points characteristic of each of the sulfide components which are present in substantial amounts.

The base sulfide is in general responsible for the electrical characteristics of the product. Any of the usual metal sulfides can be used at the base or sulfide in the practice of the present invention. For example, staple compositions have been prepared employing mixtures of an essential sulfide and one or more sulfides of the metals such as sodium, potassium, copper, silver, cadmium, platinum, mercury, lead, antimony, molybdenum, chromium, and nickel. It has also been noted that the polysulfides of the present invention may be prepared from a mixture of two or more of the sulfides which are referred to herein as the essential sulfides in which case one of the group II metal sulfides may assume the role of the base sulfide component. Such stable products include for example calcium cadmium sulfide, calcium magnesium sulfide, zinc cadmium sulfide and mercury calcium sulfide.

#### Molybdenum sulfide

For many applications and particularly to facilitate their manufacture, the compositions of the present invention also contain from about 0.03 to 10 percent, preferably less than 1 percent by weight, of molybdenum sulfide. It has been found specifically that molybdenum disulfide acts both as a lubricant and as a binder during the pressing of the sulfide mixtures thus facilitating their manufacture. Of even greater importance for many applications is the characteristic of the molybdenum sulfide to function as a depolarizer, i. e., to aid in the depolarization of the metal leads embedded in or in contact with the sintered mixture of sulfides.

#### Sulfur

A further desirable constituent of the mixed sulfides employed in the preparation of many of

the elements of the present invention is a small amount of free sulfur introduced into the mixtures prior to pressing in an amount ranging from 0.03 to as high as 10 percent but generally not exceeding about 0.5 percent by weight. As will be pointed out more fully hereinafter, a small amount of added sulfur can be employed to aid in the stabilization of the resistance characteristics of certain of the resistance elements, particularly for D.-C. applications. When employed in larger amounts, ranging up to 10 percent by weight, the sulfur also serves to increase the over-all resistance of the elements at lower temperatures.

#### Leads

A further aspect of the present invention is the provision of leads characterized by a useful life equal to that of the sulfide body per se. Heretofore considerable trouble has been encountered in providing suitable electrical connections for sulfide resistance or semi-conducting materials. Many metals, for example, silver and copper, are readily attacked by sulfur and this attack, which includes a conversion of the metallic silver or copper to a sulfide, may continue until all of the metal is so consumed. The leads or contacts employed in the practice of the present invention possess the property of reacting only to a limited extent with free sulfur to form on the surface of the lead a thin, stable, protective film of metal sulfide which apparently prevents further reaction between the metal and the sulfur or sulfide content of the sulfide body. An example of one of the least reactive lead metals is platinum and this metal can readily be used for the manufacture of electrical elements for alternating-current applications. However, it should not ordinarily be used for accurate direct-current applications due to the fact that when so used a continuous polarization of one of the platinum leads can take place over a period of time with a gradual increase in the over-all electrical resistance of the element.

Examples of suitable leads or contacts of the type which are sulfided readily but only to a limited extent are those of molybdenum, chromium, nickel and nickel or chromium alloys. While such metals or alloys, or metal leads of steel or the like plated or coated with such metals or alloys, are at first attacked by the sulfur, the attack is not a continuing one as in the case of copper and the electrical characteristics of the elements become constant upon the formation of a stable, substantially indestructible and protective film of metal sulfide on the surface of the leads or contacts, which sulfide layer also exhibits a constant and stable electrical resistance characteristic. Leads of or surfaced with molybdenum, nickel and a nickel alloy, e. g., Nichrome (80% Ni, 20% Cr) or Chromaloy (35% Ni, 15% Cr, bal Fe), and to a lesser extent aluminum leads are preferred. All of these have the desired characteristics with regard to the freedom of complete sulfidation and disintegration. Tantalum leads are subject only to the disadvantage that it is quite difficult to form a sulfide layer sufficiently thick to act as a mechanical bond between the lead and the sintered sulfide mixture. This is also true of tungsten and thorium-coated tungsten leads. While elements in which one or both of the leads are of this type are preferably first stabilized by a polarization process which will be described more fully hereinafter, once they are so stabilized, their electrical characteristics for D.-C. applications remain constant for an indefinite period of time

and are not affected by subjection to sub-zero temperatures or to elevated temperatures below the sintering temperatures. Any of these leads may also be used for elements intended for A.-C. applications and in such cases, the polarization process may be omitted or used only to the extent necessary to obtain a good bonding of the leads to the sintered sulfide.

#### Preparation of elements

In the preparation of the polysulfides of the present invention, the metal sulfides are preferably pulverized to a finely divided state and mixed in the desired proportions. Alternately, a mixture or alloy of two metals including a group II metal may be converted to a mixture of sulfides by treatment with hydrogen sulfide or sulfur dioxide. The mixtures which must contain at least two metal sulfides, at least one of which is one of the essential sulfides are pressed to the desired form or shape. It has been found that a pressure of the order of 20,000 p. s. i. is desirable in order to obtain a product of a density such that its resistance characteristics are unaffected by further pressure. In many instances, pressure as high as 40,000 p. s. i. has been found even more advantageous.

During the mixing and the pressing of the sulfides, care should be exercised to see that the mixtures remain as free as possible of various contaminants. The dies and other equipment employed in their manufacture should also be clean as it has been found that the presence of any significant amounts of impurities makes it difficult to prepare elements having the same electrical characteristics from batch to batch.

The electrical connections in the form of leads of the type hereinbefore described are preferably pressed into contact with the mixed sulfide body during the pressing operation.

After pressing, the compacted body of mixed sulfides is preferably sintered at an elevated temperature below the melting point of the mixture. The sintering temperature will vary depending upon the composition and the intended application of the element but should ordinarily be above the operating temperature of the element. For example, for those materials which exhibit a sharp break temperature and which will be operated over a temperature range including the break temperature, the sintering temperature should at least be above the break temperature. For most compositions containing a base sulfide which in the proper proportions would give a product having a break point temperature below about 200° C., the preferred sintering temperature ranges from 200° to 400° C. and the elements are ordinarily subjected to such temperature for about one hour. Higher sintering temperatures up to 1500° C. have successfully been employed in the preparation of certain elements and in some cases it has been found that the break temperature of a given composition can be increased by sintering the material at a more elevated temperature. While the sintering step is preferred, it may be omitted in certain instances as, for example, where physical strength and a sharp break point are not required.

#### Stabilization process

In the pressed or pressed and sintered condition, the elements can satisfactorily be employed in most alternating-current applications. However, in the "pressed" or "as sintered" condition and regardless of whether some free sulfur

was added to the mixed sulfides, the electrical conductivity of the sulfide elements is a combination of ionic and electronic action.

When a direct current is first passed through such elements including contacts embedded in or encasing part of the sulfide body, there is a deposition of the free sulfur on the anode with a gradual building up of a layer of metal sulfide on the anode lead, for example, molybdenum sulfide in the case of a molybdenum anode, and a corresponding change in the over-all resistance of the element. The result is a polarization of the element in the sense that its resistance in one direction is greater than that in the opposite direction. As it has been found that when the leads are of the type hereinbefore described the formation of the sulfide on the anode ceases as soon as a protective film is formed on the lead using up the free (ionic) sulfur, one aspect of the present invention is the pre-conditioning or stabilization of such elements by a process which comprises alternately passing a direct current through the element first in one direction and then in the reverse direction until the ionic sulfur is plated out on the surfaces of both metal contacts to form a stable and indestructible film of metal sulfide. Thus the stabilization process removes the sulfur and metal ions by plating them on the leads to form a stable sulfide or sulfides. By using up all or almost all of the free ions in this process, there is obtained a stable element whose conductivity is only or mainly electronic rather than both ionic and electronic. This process can also be described either as involving a double polarization process in the sense that the leads of the element are both polarized, or as a de-polarization process in the sense that the stabilized element is symmetrically conductive.

In carrying out the stabilization process, the current is reversed a suitable number of times during the stabilization treatment and the treatment is continued up to, for example, about 8 hours or until the resistance of the element is constant and the same in both directions. During the stabilization process, it has been found that the metal sulfide formed on the lead during the passage of a current in one direction is not removed or otherwise affected by the reversal of the current so that after this polarization has been completed and the ionic sulfur plated out, the stabilized elements can be employed in any direct-current circuit without consideration being given the question of direction of current flow.

A further and important advantage of this stabilization treatment is that the migration of sulfur to the vicinity of the contacts and the formation of the metal sulfide layer on the contact surfaces results in an anchoring of the contacts in or to the sintered sulfide mixture giving improved electrical and mechanical bonding and decreased contact resistance between the leads or contacts and the sulfide bodies.

In a preferred method of polarizing the electrode or electrodes in the manufacture of the stable sulfide elements, a D.-C. current of reasonably high density, e. g. 5-200 amps./sq. in. at the smaller electrode is conducted through the element while the element is held at a temperature where the resistance is low or at a minimum value. Sulfur ions are conducted to the anode and deposit thereon to form a good bond between the electrode (anode) and the semi-conducting sulfide material. By reversing the polarity and making the other lead the anode before all of

the sulfur is plated out on the first lead, it is possible to build a sulfide film on the other lead also and cause a similarly good bond to form. By varying the time of operation in each polarity, it is possible to control the amount of sulfide film formed between each lead and the semi-conducting sulfide in a manner such that the resistance of the element is the same for both polarities.

The best time schedule for the treatment will depend upon the relative areas of the two electrodes. For example, for an element in which the embedded surface areas of the two leads are about the same, the current is merely reversed a suitable number of times until the element has a constant resistance in both directions. On the other hand when the embedded area of one lead is greater than that of the other lead, it may be desirable during the first cycle of operations to proportion the times so that the lead with the greatest area is the anode for a comparatively longer time. For example, in processing an element such as shown in Fig. 4 in which the case is the larger lead or contact, the case is first made the anode for one hour and the lead having about one-tenth the area of the case is made the anode for ten minutes. Thereafter the current is reversed about every ten minutes for a total of eight hours, about every one-half hour for the next four hours and every hour for the next four hours. During this time the ammeter is checked and the current flowing in each polarity noted, and the times varied to get a product having the same resistance in both directions. When the element is fully depolarized, the current flowing should be of the same value in either polarity with the temperature constant. The total time is dependent also upon the amount of free (ionic) sulfur in the element.

When molybdenum disulfide is present in the mixture it appears to act as a depolarizer in the sense that it polarizes in the opposite direction from any of the other metal sulfides. For example, with nickel or nickel alloy leads, a molybdenum sulfide film forms on the lead in combination with the nickel sulfide of the lead material. The depolarizing effect of the molybdenum sulfide is a general one and is independent of the remaining sulfide or sulfides in the composition.

The effect of molybdenum sulfide in the polarization phenomena may best be understood by considering the electrical characteristics of two elements differing only in the fact that one contains a small amount of molybdenum sulfide and the other no molybdenum sulfide. Two such elements would otherwise consist of about 25 percent calcium sulfide, 75 percent silver sulfide and a small amount of free sulfur with molybdenum leads embedded at opposite ends of the elements.

When a D.-C. current is passed for a short time in one direction through these two elements at a temperature of 180° C., as in the first step of the stabilization process, and the resistance values of the elements on D.-C. current thereafter measured in both directions at the elevated temperature, it will be found that the element containing no molybdenum sulfide will have a resistance of, for example, 1,000 ohms in the direction of flow of the current during the polarization step and will have a high resistance in the neighborhood of 100,000 ohms in the opposite polarity. On the other hand, at the same elevated temperature, the element containing molybdenum sulfide will be found to have a re-

sistance of about 1,000 ohms in the first direction and a very low resistance of, for example, 2 ohms in the opposite direction.

If the polarizing current is thereafter passed through these two elements in the opposite direction, no substantial change in the resistance values of the element containing no molybdenum sulfide will be noted. On the other hand, the element containing molybdenum sulfide, when subsequently tested as hereinbefore described, will show a substantial decrease in the 1,000 ohm resistance at the elevated temperature until finally, after the current passing through this element has been reversed a suitable number of times, the resistance of the molybdenum sulfide-containing element will be low and in the neighborhood of 2 ohms in either direction at any temperature above its break point.

It should be noted that before any polarization, the resistance values of both elements in both directions are the same, for example, about 1000 ohms at the elevated temperature of 180° C. and anywhere from 50,000 to 100,000 ohms depending upon the free (ionic) sulfur content at room temperature. The room temperature resistance of the molybdenum sulfide element is stabilized at the higher resistance of about 100,000 ohms by the stabilization treatment.

In order that those skilled in the art better may understand how the present invention may be carried into effect, there is set forth hereinafter by way of illustration but not by way of limitation a detailed description of certain polysulfide elements within the scope of the invention.

#### Calcium silver sulfide element

The calcium silver sulfide element is representative of the polymetal sulfide elements of the invention and the effects of changing proportions, composition, sintering temperatures, etc. will be described in detail in connection with this modification of the invention.

Calcium silver sulfide elements can be prepared which, depending upon the composition, will exhibit either a continuous or substantially continuous decrease in resistance with increased temperature or a definite break point in the temperature-resistance curve. The nature of the curve as well as the resistance of the element of any given temperature depends primarily upon the relative proportions of calcium and silver sulfide. The effects of varying the ratio of these two materials is illustrated in Fig. 6 of the drawing.

The curves plotted in this figure were obtained by varying the proportions of calcium and silver sulfides of stabilized elements prepared from mixtures containing about 1 percent molybdenum disulfide and about 1 percent sulfur. The elements were provided with either molybdenum or nickel chromium leads and, during the stabilization process, that sulfur which had not become chemically combined with the calcium silver sulfide composition was plated out on the leads in the form of metal sulfide coating.

As is the case with all of the other polysulfide elements, any of the leads described hereinbefore can be used, there being no noticeable difference in the resultant resistance characteristics of the elements. Some leads, such as those of Chromaloy may require a slightly longer time for polarization, i. e., sulfidation.

With reference to Fig. 6, it will be noted that compositions containing about 10 percent calcium sulfide have a temperature-resistance curve which is substantially a straight line. However,

as the calcium sulfide content is increased the temperature-resistance curve bulges upwardly at temperatures below 175° C. until at a composition which contains about 25 percent calcium sulfide, a curve is obtained which is characterized by a maximum break point, i. e., a maximum drop in resistance over a relatively narrow temperature range. It is to be noted that during this entire increase in the calcium sulfide content from 10 to about 25 percent, the resistance of the compositions at and above 175° C. is extremely small and for all practical purposes zero. In fact, the temperature of 175° C. represents the break point of those calcium silver sulfide elements having a calcium sulfide content of from about 20 to 30 percent by weight.

With further increase in the calcium sulfide content, the low temperature-resistance of the element remains substantially the same as the low temperature resistance of the compositions containing less than 30 percent calcium sulfide. The high temperature resistance of such calcium sulfide rich mixtures gradually increases with increased calcium sulfide content and the temperature-resistance curve again approaches a straight line.

In general, it appears advisable to employ calcium silver sulfide compositions containing at least 10 percent and not over 60 percent calcium sulfide. Pressed mixtures of calcium and silver sulfide containing less than 10 percent of the calcium sulfide are physically weak, while those containing over 60 percent have resistance values of 1000 to 2000 ohms even at the more elevated temperatures.

With regard to the effect of the sulfur content of the stabilized elements, it appears that sulfur affects only the low temperature-resistance values, i. e., the electrical resistance of the elements below the break-point temperature. In Fig. 7 there is plotted a number of curves indicating roughly the change in the low temperature-resistance values of calcium silver sulfide elements containing 25% calcium sulfide, and from 0 to 10 percent added sulfur. In general, about 3 percent sulfur is preferred in order to assure an ample supply of sulfur ions for the depolarization of the leads and to form a coating of metal sulfide on these leads sufficient to provide a good mechanical and electrical bonding layer between the sulfide composition and the leads.

It has also been found that the resistance characteristics of the elements of the present invention can be further modified without affecting their stability by the addition thereto of minor proportions, for example, up to 30 percent by weight of powdered metal. For example, the addition of up to 30 percent powdered silver to the calcium silver sulfide compositions results in a product, the resistance value of which decrease extremely rapidly with increased temperature. The temperature-resistance curve of a stabilized element containing 18 parts calcium sulfide, 80 parts silver sulfide, 18 parts molybdenum sulfide, 1 part sulfur, and 20 parts powdered silver is shown in Fig. 8. The resistance value of this element decreases to its lowest value at a temperature of about 175° C.

Many of the alloys of a metallic sulfide and calcium sulfide are greatly affected by the sintering temperature. This is particularly true of those which are sintered below 600° C. Calcium silver sulfide is in this group. When sintered at 400°, the calcium silver sulfide has a permanent and characteristic resistance curve and shows very little, if any, aging effect after the

first week. However, when these compositions are sintered at only 300°, there is an appreciable aging effect, but after about one week, standing at room temperature, such elements take on a permanent temperature-resistance characteristic which is the same as that obtained immediately by sintering the elements at about 400° C. When the calcium silver sulfide elements are sintered at temperatures substantially above 400° C., the characteristics of the resistance curve are changed so that the resultant elements will not have as low a resistance value when heated above the break-point temperature as when sintered at 400° C. In general, in the preparation of most of the elements of this invention compounded to have a definite break point, it has been found desirable to sinter at a minimum temperature substantially twice the break-point temperature in degrees centigrade.

It has previously been noted that break-point temperature of the calcium silver sulfide mixtures is approximately 175° C. This temperature results from the presence of the silver sulfide since substantially the same break temperature is obtained by substituting any of the other group II metal sulfides, such as zinc, cadmium or magnesium sulfide, for the calcium sulfide component.

#### *Calcium cadmium sulfide elements*

This is an example of an element of the present invention comprising two of the essential sulfides, specifically, a mixture of cadmium sulfide and calcium sulfide. A composition containing 50 percent cadmium sulfide, 40 percent calcium sulfide, 5 percent molybdenum disulfide and 5 percent added sulfur exhibits a break point of 550° C. The cadmium calcium sulfide elements are preferably sintered at temperatures up to 1200° C. for maximum freedom from aging. In general, satisfactory elements can be obtained from compositions containing from 40 to 90 percent cadmium sulfide, 10 to 60 percent calcium sulfide, 0.03 to 10 percent molybdenum disulfide and 0.03 to 10 percent excess sulfur. The sulfur may also be omitted particularly when it is not required for sulfiding the leads.

#### *Molybdenum calcium sulfide elements*

Particularly good elements are those in which the molybdenum disulfide is the base sulfide as well as the binder and depolarizer. One such element is prepared from calcium sulfide, molybdenum sulfide and, if desired, some added sulfur. These two or three materials are mixed in the usual manner, pressed at a high pressure, and thereafter sintered at a temperature up to about 1200° C.

The elements containing molybdenum sulfide as the base sulfide are representative of those in which the break-point temperature is affected by composition. For example, an element containing a sintered mixture of about 91.7 percent calcium sulfide and 8 percent molybdenum disulfide, and 0.3 percent sulfur exhibits a definite break in the temperature-resistance curve at about 250° C. The break temperature increases with increased molybdenum disulfide content. An element containing 55 percent calcium sulfide, 35 percent molybdenum disulfide, and 10 percent sulfur exhibits a break point of about 350° C. The break point is independent of the sulfur or excess sulfur content within the range of 0 to 10 percent added sulfur and appears to be entirely dependent upon the relative proportions of the essential sulfide and molybdenum sulfide.

Preferably, the molybdenum sulfide is present in only a minor proportion. The reason for this is that when the content of molybdenum sulfide substantially exceeds 35 percent of the composition, the high temperature stability of the element is impaired and when an element containing more than 35 percent molybdenum sulfide is substantially overheated, a permanent change in the resistance characteristics in one direction will result. Elements containing mercury sulfide as the base sulfide are another example of elements in which the quantity of the base sulfide is kept low, however, for a different purpose. With a mercury sulfide element, a high dilution of the mercury sulfide is desirable to prevent spontaneous combustion or explosion of the mixture.

#### *Other sulfides*

Except for those compositions in which the break point temperature is dependent upon proportions of base sulfide as is the case with the molybdenum sulfide element, it is necessary to change the base sulfide in order to obtain elements having different break points. The following is the list of a number of suitable sulfides which have been used, the list including the approximate break-point temperatures noted for mixtures of the designated sulfide with one of the essential sulfides.

|                    | Approx. Break Point Temp. |
|--------------------|---------------------------|
| Sodium sulfide     | 15° C.                    |
| Potassium sulfide  | 20° C.                    |
| Mercury sulfide    | 25° C.                    |
| Lead sulfide       | 80° C.                    |
| 35 Copper Sulfide  | 90° C.                    |
| Silver Sulfide     | 175° C.                   |
| Molybdenum sulfide | 250°-400° C.              |
| Nickel sulfide     | 400° C.                   |
| Antimony sulfide   | 400° C.                   |
| 40 Cadmium sulfide | 550° C.                   |
| Barium sulfide     | 800° C.                   |
| Zinc sulfide       | 800° C.                   |

Mixtures of chromium sulfide and calcium sulfide yield a product having a high and constant resistance at temperatures of from 0° C. to 900° C., i. e., products having a zero temperature coefficient of resistance. Platinum sulfide as the base sulfide gives a material having a high negative coefficient below about 150° C., a rather low coefficient from 150° to 280° C., and a rather sharp break in the resistance values at about 280° C.

In general, it may be stated that the calcium sulfide (or its equivalent essential sulfide) is usually employed in a minor proportion and preferably from 15 to 25 percent when a maximum break point is desired. Exceptions to this general statement are the molybdenum sulfide, mercury sulfide and chromium sulfide elements and the 60 elements containing zinc sulfide as the essential sulfides. As to the last mentioned sulfide, best results have been noted with the silver zinc sulfides when the zinc sulfide content was about 50 percent with satisfactory elements being obtained from mixtures containing as much as 70 percent zinc sulfide.

While the invention has been specifically described with reference to sintered mixtures of one essential sulfide and one base sulfide (except for small amounts of molybdenum sulfide), it is to be understood that mixtures comprising more than one base sulfide and one or more essential sulfides are also within the scope of the invention. Such mixtures will in most cases exhibit temperature-resistance curves which are, on the whole,

a composite of the curves of the separate base sulfides.

In all of the compositions, the essential sulfide, particularly the calcium sulfide, functions not only to impart stability to the mixture but also as a binder. It is for this latter reason that an essential sulfide content of at least from 3 to 5 percent and preferably 10 percent is desirable. However, in spite of the binding effect of the calcium sulfide in most cases it has been found highly beneficial also to employ at least 0.3 percent molybdenum sulfide which not only lubricates the mixture during the pressing operation but also is far superior to any of the essential sulfides in its binding properties.

With further reference to the stabilization process, this treatment has been found to have three distinct and desirable effects. The most important is probably a stabilization of the resistance characteristics of the element although from the mechanical standpoint, the anchoring of the leads as a result of the formation of the sulfide film thereon is also of substantial importance. In addition, any free or unattached sulfur ions which have not been removed by evaporation or chemically combined with the sulfides during the sintering process are plated out during the stabilization process thereby using up any excess sulfur so that the action of the element is mainly electronic rather than a combination of ionic and electronic. The term excess sulfur as used here refers not so much to the total amount added to the mixture prior to pressing as to that part which has not entered into chemical combination with the metal sulfides to form either a metal sulfide-sulfur complex or a lower metal sulfide; in other words, the sulfur above that required for the stoichiometric compositions.

In this connection, the stabilization process is not limited to sulfide resistance elements but is broadly applicable to other non-metallic, inorganic semi-conductors, such as the resistance elements comprising one or more metal oxides, selenides, tellurides, or the like with regards to which the art has been continuously concerned with both the problem of anchoring leads in such elements and with the problem of obtaining stable elements. By the stabilization or polarizing process described herein, the free ions present in the resistance materials can be plated out on selected leads of a metal or alloy which readily reacts with these ions to form a stable compound. There is thus obtained not only a temperature stable element but also one within which the leads are firmly anchored or secured to the resistance material as a result of the formation of the stable compound or compounds on the leads. As in the case of the sulfide elements, it may also be desirable to deliberately have present in the element composition a small amount of an element or compound which is the source of free or uncombined ions that are free to migrate to the leads during the polarization treatment and combine therewith to form a stable compound or layer. This may be accomplished by adding an ion-providing element or compound to the material prior to the pressing or forming of the element or in the case of the oxides, by sintering or firing the elements in an oxygen or an oxygen rich atmosphere.

Also during the stabilization process, any free metal present in those elements prepared from mixtures including added free metal reduces the other metallic sulfides in the mixtures so that the alloy becomes less than a stoichiometric mix-

ture or compound. In other words with added silver the alloy becomes a silver rich alloy.

The elements of the present invention can be used in any of the various applications where a thermally responsive resistance element is required. They have the added advantage over the previously known thermistor elements of being substantially insensitive to changes in voltage and of being fast enough in response to changes in temperature in the neighborhood of their break points to be able to operate alternating-current relays directly.

What I claim as new and desire to secure by Letters Patent of the United States is:

15. 1. A stable electric resistance unit comprising a body of resistance material consisting essentially of a pressed mixture of metal sulfides including (1) from 3 to 95 per cent of a sulfide of a metal of group II of the periodic table selected from the class consisting of magnesium, calcium, zinc, cadmium, barium and mercury, and (2) molybdenum sulfide and metal leads electrically connected to said body of resistance material.
- 20 25. 2. A stable resistance unit composed of a body of resistance material consisting essentially of a compressed, sintered mixture of metal sulfides including at least 0.03 per cent molybdenum sulfide and from 10 to 60 per cent of at least one sulfide of a metal of group II of the periodic table and metal leads electrically connected to said body of resistance material.
- 30 35. 3. A stable, thermally sensitive resistance unit composed of a body of resistance material consisting of a compressed, sintered mixture of a plurality of metal sulfides including molybdenum sulfide, from 3 to 95 per cent of a sulfide of a metal of group II of the periodic table and a substantial portion of a third metal sulfide and metal leads electrically connected to said body of resistance material.
- 40 45. 4. A stable, thermally sensitive resistance unit composed of a body of resistance material comprising a pressed and sintered mixture of metal sulfides essentially including from about 0.03 to 35 percent molybdenum disulfide and from 3 to 95 percent of a sulfide of a metal of group II of the periodic table and metal contacts electrically connected to said body of resistance material, at least one of said contacts being molybdenum.
- 50 55. 5. A stable polysulfide resistance element comprising a body of resistance material consisting of a sintered compressed mixture of at least two metal sulfides including from 10 to 95 percent of at least one sulfide of a group II metal and at least 0.03 percent molybdenum sulfide and metal contacts electrically connected to said body, at least one of said contacts being a molybdenum contact embedded in said body.
- 60 65. 6. A stable, thermally sensitive resistance element comprising a body of resistance material consisting of a compressed, sintered mixture of metal sulfides including from about 0.03 to 10 percent molybdenum sulfide, 10 to 60 percent of a sulfide of a group II metal and a substantial portion of a third metal sulfide and metal contacts electrically connected to said body.
- 70 75. 7. A stable resistance element comprising a body of resistance material consisting of a compressed sintered mixture of 0.03 to 10 percent molybdenum disulfide, 40 to 90 percent cadmium sulfide and 10 to 60 percent calcium sulfide and metal contacts electrically connected to said body.

8. A stable thermistor consisting essentially of a body of resistance material consisting of a pressed, sintered mixture of a plurality of metal sulfides including molybdenum sulfide, 3 to 95 percent of a group II metal sulfide and silver sulfide and metal contacts electrically connected to said body.

9. A stable thermistor consisting essentially of a body of resistance material consisting of a compressed sintered mixture of from 0.03 to 10 percent molybdenum disulfide, 15 to 35 percent calcium sulfide, balance substantially all silver sulfide and metal contacts electrically connected to said body.

10. A stable thermistor composed of a body of resistance material consisting of a pressed sintered mixture of metal sulfides consisting of from 0.03 to 10 percent molybdenum sulfide, 15 to 25 percent calcium sulfide and balance silver sulfide and metal contacts electrically connected to said body, at least one of said contacts being a molybdenum contact embedded in said body.

11. A stable resistance element comprising a body of resistance material consisting of a sintered mixture of .03 to 10 percent molybdenum sulfide, 10 to 60 percent of a sulfide of a group II metal, silver sulfide, and a small amount of sulfur and metal contacts electrically connected to said body.

12. A stable thermistor element comprising a body of resistance material consisting of a pressed, sintered mixture of at least 0.03 percent molybdenum sulfide, from 10 to 60 percent of a sulfide of a group II metal, silver sulfide, a small amount of sulfur and a minor portion of powdered silver and metal contacts electrically connected to said body.

13. A stable thermistor element comprising a body of resistance material consisting of a pressed sintered mixture of at least 0.03 percent molybdenum sulfide, 3 to 95 percent zinc sulfide and a third metal sulfide and metal contacts electrically connected to said body.

14. A stable thermistor element comprising a body of resistance material consisting of a sintered mixture of at least 0.03 percent molybdenum sulfide, 3 to 95 percent cadmium sulfide and a third metal sulfide and metal contacts electrically connected to said body.

15. A stable thermistor comprising a body of resistance material consisting of a sintered mixture of at least 0.03 percent molybdenum sulfide, 3 to 95 percent calcium sulfide and a third metal sulfide and metal contacts electrically connected to said body.

16. A stable resistance element comprising a body of resistance material consisting of a sintered mixture of molybdenum sulfide, chromium sulfide and 3 to 95 percent calcium sulfide and metal contacts electrically connected to said body.

17. A stable resistance unit comprising a body of resistance material consisting essentially of a sintered mixture of metal sulfides including molybdenum sulfide and 3 to 95 percent of a sulfide of a group II metal and metal leads electrically connected with said resistance material.

18. A stable resistance unit comprising a body of resistance material consisting of a sintered mixture of sulfides including at least 0.03 percent molybdenum sulfide and 3 to 95 percent of a sulfide of a group II metal and molybdenum contacts electrically connected to said body.

19. A stable resistance unit comprising a body of resistance material consisting of a compacted mixture of sulfides including a small amount of

molybdenum sulfide and 3 to 95 percent of a sulfide of a group II metal and metal leads electrically connected to said body including a molybdenum lead embedded in said body in electrical contact therewith, said lead having thereon a film of molybdenum disulfide.

20. A stable resistor unit comprising a sintered, body of resistance material consisting of a sintered compressed mixture of metal sulfides including a small amount of molybdenum sulfide, 3 to 95 percent of a sulfide of a group II metal and a third metal sulfide, and metal leads electrically connected with said body, at least one of said leads having a nickelous surface and having a sulfide layer on the surface thereof in contact with said body.

21. A stable resistance unit comprising a body of resistance material consisting of a sintered compressed mixture of metal sulfides including a small amount of molybdenum sulfide, 10 to 60 percent of a sulfide of a group II metal and a major portion of a third metal sulfide and metal leads including a sulfide-coated metal lead electrically connected with said sulfide-coated body, said lead being an alloy of 35 percent nickel, 15 percent chromium, balance substantially iron.

22. A stable resistance unit comprising a sintered compacted body of resistance material consisting of a mixture of metal sulfides including a small amount of molybdenum sulfide, 3 to 95 percent of a sulfide of a group II metal and a major portion of a third metal sulfide and metal leads electrically connected with said body, one of said leads being of a nickel-chromium alloy and having a sulfide coating thereon.

23. The method of preparing a stable sulfide resistance element which comprises forming a mixture of at least two metal sulfides including at least 0.03 percent molybdenum sulfide and 3 to 95 percent of at least one sulfide of a group II metal, pressing said mixture into contact with a metal lead which will react with sulfur to form a stable sulfide film thereon but which does not sulfide to the point of disintegration of the lead, sintering the sulfide mixture and thereafter passing a current through said mixture and lead to form a sulfide layer on said lead.

24. The method of obtaining a good mechanical and electrical connection between a polysulfide resistance element and an electrical contact element therefor which comprises pressing a powdered mixture of the sulfides comprising the polysulfide element into contact with the contact element with a portion of one of said elements encompassing a portion of the other of said elements, heating the resultant product to sinter the polysulfide mixture and thereafter passing a direct current through the product to build up a sulfide film on the surface of the contact element in engagement with the polysulfide element.

25. The method of claim 24 wherein the mixture of sulfide is pressed into contact with a contact element in the form of a wire having an end portion thereof embedded in the pressed mixture of sulfides.

26. The method of claim 24 wherein the mixture of sulfides is pressed into contact with a contact element in the form of a cap enclosing a portion of the pressed mixture of sulfides.

27. The method of obtaining a good mechanical and electrical connection between a resistance element comprising a sintered mixture of metal sulfides and a metal lead which comprises pressing a powdered mixture of the sulfides including at least 0.03 percent molybdenum sulfide

and 3 to 95 percent of a sulfide of a group II metal and a small amount of sulfur into contact with a metal lead which has the property of reacting with sulfur to form a stable protective sulfide film on the surface thereof, heating the resultant product to a temperature sufficient to sinter the sulfide mixture, and passing a direct current through said product to form on the surface of the lead in contact with the sintered sulfide mixture a layer of metal sulfide, said layer forming a good mechanical bond between said lead and said mixture.

28. The method of claim 27 in which the sintered sulfide mixture is held at a temperature at which the electrical resistance is low during passage of the direct current.

29. The method of claim 28 wherein the portion of the lead in contact with the sulfide mixture is molybdenum.

30. The method of claim 27 in which the sintered sulfide mixture is held at a temperature at which the electrical resistance is low during passage of the direct current and wherein the portion of the lead in contact with the sulfide mixture comprises nickel.

31. The method of claim 27 in which the sintered sulfide mixture is held at a temperature at which the electrical resistance is low during passage of the direct current and wherein the portion of the lead in contact with the sulfide mixture is an alloy essentially containing nickel and chromium.

32. The method of claim 27 in which the sintered sulfide mixture is held at a temperature at which the electrical resistance is low during passage of the direct current and wherein the portion of the lead in contact with the sulfide mixture is an alloy consisting of nickel and chromium.

33. The method of stabilizing the resistance characteristics of a sulfide resistance element containing at least 0.03 percent molybdenum sulfide and 3 to 95 percent of a sulfide of a metal of

group II of the periodic table, which comprises passing a direct current through said element while holding the element at a temperature at which its electrical resistance is at a minimum value.

34. The method of forming a stable resistance element which comprises forming a mixture of a plurality of metal sulfides including molybdenum sulfide, 3 to 95 percent of a sulfide of a group II metal and a small amount of sulfur, pressing said mixture into contact with metal leads which will react with sulfur to form a stable surface layer of metal sulfide, sintering the pressed sulfide mixture and thereafter passing a direct current between said leads through the sintered mixture while the sintered sulfide mixture is held at a temperature above that at which its electrical resistance approaches a minimum, periodically reversing the direction of current flow, and continuing said process until the ionic sulfur remaining in the sintered mixture is deposited on said leads to form on the surfaces thereof sulfide films which mechanically and electrically bond and connect said leads to the sintered sulfide mixture.

FREDERIC R. QUINN.

#### REFERENCES CITED

The following references are of record in the 30 file of this patent:

#### UNITED STATES PATENTS

| Number    | Name            | Date          |
|-----------|-----------------|---------------|
| 959,068   | Phillips        | May 24, 1910  |
| 1,820,591 | Andre           | Aug. 25, 1931 |
| 2,197,115 | Randolph et al. | Apr. 16, 1940 |

#### FOREIGN PATENTS

| Number  | Country       | Date          |
|---------|---------------|---------------|
| 144,608 | Austria       | 1936          |
| 360,920 | Great Britain | 1931          |
| 367,790 | Great Britain | Feb. 15, 1932 |
| 701,172 | France        | 1931          |